

June 20, 1939.

R. W. KENT

2,162,778

MANUFACTURE OF PILE FABRICS

Filed May 2, 1936



## UNITED STATES PATENT OFFICE

2,162,778

## MANUFACTURE OF PILE FABRICS

Raymond W. Kent, Newton Highlands, Mass.

Application May 2, 1936, Serial No. 77,537

9 Claims. (Cl. 28—1)

This invention relates to the manufacture of pile fabrics in which the pile is adhesively attached to one surface of a fabric backing, and has particularly to do with the provision of improved methods of preparation and treatment of the pile or flock to be attached to said backing, though it also includes the further steps in the manufacture of such pile fabrics. The invention is especially useful in the manufacture of pile of 5 substantially uniform length, for the flock if too long and non-uniform will not sift readily and will ball up in the flock-applying process or mat unevenly on the adhesively coated fabric or other backing and, if too short, it will not embed deeply 10 enough in the adhesive to provide adequate wear resistance.

Heretofore cotton and rayon as made and adhesively applied by the suede fabric trade to rubber coated fabric have been relatively short, 20 for example,  $\frac{1}{64}$ "— $\frac{1}{25}$ " long, and ground either in a high speed grinder with resultant injury to the fibres, and the production of uneven lengths, much dust and fibre loss, or cut by a guillotine device which is relatively slow and costly, and, as, 25 a consequence, guillotine cutting has not been generally used. In the dry grinding as practiced, the fire or explosive hazard is great and many serious dust explosions have resulted, for the fibre, cotton or rayon for example, ground at high speed 30 is extremely fine and when thoroughly mixed with air (oxygen) an ideal combination is presented for an explosion, should a spark by chance be available.

It is the object of this invention to provide an 35 improved method of providing a clean and relatively dustless fibre in substantially uniform short lengths and without injury to or mashing of the ends of the same. The method includes the cutting and treating of fibres such as cotton, rayon, 40 or animal fibres such as wool, mohair, rabbit's hair, silk, etc., to provide a flock, and all of which fibres, it has been discovered, may in accordance with this invention be successfully cut to substantially uniform lengths by passing the fibres, 45 as hereinafter described, in a fluent liquid carrying medium through a cutting device.

All of the above mentioned fibres, with the exception of cotton, may be wet-cut in an aqueous carrying medium, but with cotton fibre it has been 50 found preferable, to prevent hydration, to cut it in some freely fluent non-aqueous liquid medium, for example, kerosene, vegetable oil, or other suitable non-hydrating liquid carrying medium compatible with the fibre. It is found in practice 55 that with the wet-cutting of the fibres the ends

thereof are substantially as cleanly cut as in the guillotine method and are not injured,—not crushed or mashed, as in the dry grinding method. Moreover, a uniform and straighter fibred flock is secured, presumably because of the tendency of 5 the long fibres to more or less align themselves in the fluent or freely moving body of liquid as in the apparatus which I preferably employ. Another outstanding advantage of my method of treatment is that the material thus secured is 10 much cleaner,—free from dust. The cleaning may be enhanced by any suitable cleaning fluid or by the presence of a small amount of soap. The washing and scrubbing action produces a 15 flock freer from dirt which dirt, being either 15 lighter or heavier than the fibres, tends to separate from the fibres and thus, if desired, may be readily removed from the liquid. Thus there is produced a clean short cut flock of uniform length (for example,  $\frac{1}{64}$ " to  $\frac{1}{4}$ ") the fibres of which retain substantially their uniform physical and chemical characteristics.

In the drawing, which illustrates the method and a form of apparatus suitable for practicing the same,—the figure shows a front elevational 25 view with various parts broken away for purposes of clarity.

Referring to the drawing there is shown at 1 a mixing tank having therein a stirring impeller 2, which tank is connected through a valve 3 to a 30 cutting device generally designated at 4, said device comprising a frusto-conical cutter mounted for rotation as shown having upon its exterior a series of helical blades 5 which are rotated in closely adjusted relation with reference to a fixed 35 series of longitudinal blades 6, so as to provide therewith a shearing cut. The fluent mass of long fibres upon being mixed in the liquid in the tank 1 is passed through the cutting device 4 wherein the fibres are cut to shorter lengths and thence through the valve 7 into a heat-jacketed lower tank 8 having therein an impeller 9 from which the flock thus cut to a shorter length may either be withdrawn through the valve 10, or, if necessary, to shorten it still further, pumped 45 by means of the gear pump 11 and return line 12 back into the tank 1 from which it may again be passed through the cutting device.

As a specific example of the treatment of fibre, say rayon fibres or thread, which it is desired to 50 reduce to a length of say  $\frac{1}{25}$ " or less, the following is given,—to the water in which there is added rayon fibre in the amount of .1 ounce per pound of water and the cutting is carried on for the required period to reduce the fibre to said length,

the period varying somewhat depending upon the rapidity of the flow and circulation, and the setting of the moving and fixed elements of the device.

- 5 5 In addition to the reducing of the fibre to substantially uniform length, it may be and preferably is, dyed in the apparatus (preferably provided with a heat jacket as shown), thus providing a thorough mixing of the dye with the fibre 10 10 material thus colored. The dye may either be added in the first instance to the water or other liquid in the mixer (preferably water in the case of rayon or non-aqueous liquid in the case of cotton) or later added. A further advantage of 15 15 the wet-cutting in the device is that two or more previously colored flocks may be simultaneously cut, washed and combined, with or without additional dyeing, to produce a "heather effect", red and green for instance, the mixing taking place 20 20 during the cutting as herein set forth.

Though it is not essential for the successful practice of the process of this invention, particularly where only short fibres are applied, it is sometimes desirable to subject long pile or fibres 25 25 to a preliminary sizing treatment and thus temporarily render the fibres heavier, smoother and stiffer, for it has been discovered that fibres, especially the longer fibres, when rendered relatively stiff, straight and smooth, can be flocked 30 30 and applied to a backing much more effectively. The sizing may conveniently be done before the pile material is cut, and should involve the use of a size insoluble in the liquid carrying medium. For example, if the latter be kerosene, 35 35 a water-soluble size is employed, for example, gelatin, glue, dextrin, gum-tragacanth, etc., whereas if an aqueous carrying medium is used in the cutting process, a water-insoluble size is employed, for example, pyroxylin, silicate of soda, 40 40 or resins, natural or synthetic. An additional advantage of the sizing, as herein described, lies in the fact that the manufacturer may both cut and apply to the backing as one unit a thread made up of many fine filaments, for example rayon, or, 45 45 to put it another way, to cut and apply as a unit a bundle of filaments. Such bundle may be left either in bundle form, or desized and loosened, as desired. In the usual practice of the invention the cut fibres are preferably well dried and loosened 50 50 before being applied to the backing (fabric, rubber, wood, metal or other firm material) in order that they may be free and separated from one another so as to be readily applied as by sifting to the backing in generally endwise arrangement 55 55 and with the ends thereof embedded in the adhesive. Any sort of rubber or equivalent adhesive, for example, as already known and used in the art, may be employed to attach the fibres to a rubber coated base, but I preferably employ a normally liquid heat-treated rubber bonding agent as described and claimed in my application Serial No. 218,971, filed July 13, 1938. Whatever type of adhesive be employed, the fibres are deposited therein, as well known in the art, 60 60 and thus the heat-treated rubber or other form of rubber adhesive is either permitted to solidify or rendered solid as required so that the fibres are firmly held to the backing by vulcanized rubber. After the vulcanizing step, the size, if employed, 65 65 may be washed out with an appropriate liquid harmless to the adhesive. If desired, the product can also be further dyed after removing the size, but before drying.

Having described my invention what I wish 70 70 to claim and secure by Letters Patent is:—

1. The process of making a pile fabric comprising mixing separated long fibres in a liquid, carrying said fluent liquid mass to a cutter, wet-cutting said fibres to a substantially uniform and shorter length, and while the fibres are still wet, dyeing the same, drying the fibres thus cut and dyed and then embedding the ends of the fibres in a liquid adhesive fibre-to-base bonding agent. 5

2. The process of making a pile fabric comprising mixing separated long fibre units in a liquid, carrying said fibre-containing liquid to a cutter, wet-cutting said fibres to a substantially uniform and shorter length, and, while the fibres are still wet, dyeing the same, drying the fibres thus cut and dyed, and then embedding the ends 15 15 of the fibres in a normally liquid adhesive fibre-to-base bonding agent to attach the fibres to a base material.

3. The process of making a pile fabric comprising sizing long fibres, mixing said fibres in a liquid, carrying said fibre-containing liquid to a cutter, wet-cutting said fibres to a substantially uniform and shorter length, and, while the fibres are still wet, drying the fibres thus sized and cut, and then embedding the ends of the fibres in 25 25 a liquid adhesive fibre-to-base bonding agent to attach the fibres to a base material.

4. The process of making a pile material which consists in wet-cutting unrestrained long fibre units of the class described, freely floatant in a liquid carrying medium, to a flock of shorter and substantially uniform length, drying said cut fibres, and thereafter embedding ends of the fibres in a liquid adhesive fibre-to-base bonding agent to attach the fibres to a base material. 35

5. The process of making a pile material which consists in repeatedly wet-cutting unrestrained separated long fibres of the class described, mixed in and carried by a liquid medium, to a flock of shorter and substantially uniform length, drying 40 40 said cut fibres and thereafter embedding ends of the fibres in a liquid adhesive fibre-to-base bonding agent to attach the fibres to a base material.

6. The process of making a pile coat having fibres end-embedded in a fibre-to-base bonding agent, comprising mixing separated long fibre units of the class described in a liquid carrying medium to provide a fluent liquid mass containing unrestrained fibre units, passing said fluent mass between cutting edges, wet-cutting said 50 50 fibres to a flock of shorter and substantially uniform length, drying said cut fibres, and thereafter embedding ends of the fibres in a liquid adhesive fibre-to-base bonding agent to attach the fibres to a base material. 55

7. The process of making a pile material having fibres end-embedded in a fibre-to-base bonding agent comprising mixing separated long fibre units of the class described in a liquid carrying medium to provide a fluent liquid mass containing unrestrained fibre units, passing said fluent mass between cutting edges, wet-cutting said 60 60 fibres to a flock of shorter and substantially uniform length, and at some stage of the process dyeing the fibres, and thereafter embedding ends of 65 65 the fibres in a liquid adhesive fibre-to-base bonding agent to attach the fibres to a base material.

8. The process of making a pile material comprising mixing separated long fibre units in a liquid to provide a fluent liquid mass containing 70 70 unrestrained fibre units, flowing said fluent mass between cutting edges, wet-cutting said fibres to a shorter and substantially uniform length and at some stage of the process dyeing and sizing the fibres and thereafter drying the fibres and embed- 75

ding ends of the fibres in a liquid adhesive fibre-to-base bonding agent to attach the fibres to a base material.

ting said fibres to a substantially uniform and shorter length, drying the fibres and then embedding the ends of the fibres in a liquid adhesive fibre-to-base bonding agent.

9. The process of making a pile fabric comprising mixing separated long fibres in a liquid, carrying said fluent liquid mass to a cutter, wet-cut-

5

RAYMOND W. KENT.